

# UNITED STATES PATENT OFFICE.

MILTON W. FRANKLIN, OF SCHENECTADY, NEW YORK, ASSIGNOR TO GENERAL ELECTRIC COMPANY, A CORPORATION OF NEW YORK.

## PROCESS OF PLATING METALS.

1,037,887.

Specification of Letters Patent. Patented Sept. 10, 1912.

No Drawing.

Application filed August 4, 1911. Serial No. 642,267.

To all whom it may concern:

Be it known that I, MILTON W. FRANKLIN, a citizen of the United States, residing at Schenectady, county of Schenectady, State 5 of New York, have invented certain new and useful Improvements in Processes of Plating Metals, of which the following is a specification.

My invention comprises a process for electrolytically coating non-conducting surfaces with metal.

The method formerly in use for coating non-conducting material, such as glass, with metal consists in first covering the material 15 to be coated with a varnish, such as copal or shellac. The varnish furnished a sticky surface which was coated with graphite, and was then made the cathode in a plating bath. In the finished product the metal film is attached to the glass, or other vitreous surface 20 only by means of the varnish, which renders the articles thus plated unfit for use at high temperatures. Even at ordinary room temperature the metal coating can be easily 25 peeled off.

I have discovered that when the non-conducting surface is coated with an adhesive which is permeable, and preferably also soluble, in the plating electrolyte, and a conducting layer is applied as usual, the plated film adheres very firmly to the surface upon 30 which it is applied. To render the film of adhesive conducting, I prefer to use, in a finely divided state, the metal to be plated, 35 or a metal with which it will readily unite and incorporate the same, as by rubbing, into the adhesive film. During the plating process, metal is deposited on all sides of each particle.

As a suitable material for the adhesive 40 coating, I may mention gum arabic, fish glue, water shellac, gum dammar, or gum tragacanth. An aqueous, or other suitable solution of the gum is applied in a very 45 thin layer upon the non-conducting surface to be coated. The surface is sprinkled with a very fine powder of metal, preferably of the metal to be plated, for example, copper. The copper powder is then rubbed into the 50 film of adhesive. When the surface thus prepared is plated in the ordinary way, each grain of the original metal powder is coated with metal and the minute quantity of ad-

hesive is practically dissolved out leaving a coating of pure metal. If any portion of the 55 adhesive remains, it is probably incorporated with the metal.

The metal coating applied in this manner is very strong and can be removed from a smooth glass or other vitreous surface only 60 with the greatest difficulty. Its appearance, when viewed through the glass is similar to that of a mirror of the metal.

This process is particularly useful for coating vitreous or other non-conducting 65 surfaces of condensers, ozone tubes and other electrical apparatus which are frequently operated at an elevated temperature.

What I claim as new and desire to secure by Letters Patent of the United States, is,

1. The process of preparing non-conducting surfaces to receive an electrolytic deposit which consists in covering said surface with a film of adhesive material permeable with respect to the electrolyte in which the 75 object is to be plated, incorporating conductive material into the adhesive film and electro-plating a metallic coating thereon.

2. The process of preparing a non-conductive surface to receive an electrolytic deposit which consists in covering said surface with a thin layer of adhesive material permeable and soluble in the solution which will subsequently form the plating bath, 80 working a conductive powder into said adhesive and electro-plating a metallic coating 85 thereon.

3. The process of preparing vitreous surfaces to receive an adherent electrolytic deposit of metal which consists in applying a 90 thin coating of water soluble gum upon said surface, and incorporating into said coating a finely powdered conducting material.

4. The process which consists in coating a non-conducting surface with a soluble 95 gum, incorporating a finely powdered conducting metal into said gum, and utilizing the resulting conductive layer as cathode in a plating bath.

In witness whereof, I have hereunto set 100 my hand this 3rd day of August, 1911.

MILTON W. FRANKLIN.

Witnesses:

BENJAMIN B. HULL,  
HELEN ORFORD.